



US005503644A

# United States Patent [19]

Graiff et al.

[11] Patent Number: 5,503,644

[45] Date of Patent: Apr. 2, 1996

[54] **GASOLINE COMPOSITION FOR REDUCING INTAKE VALVE DEPOSITS IN PORT FUEL INJECTED ENGINES**

4,357,148 11/1982 Graiff .  
4,936,868 6/1990 Johnson .  
5,006,130 4/1991 Aiello et al. .

[75] Inventors: **Leonard B. Graiff**, Houston; **Robert P. Aiello**, Cypress; **H. Dale Millay**, Michael J. Riley, both of Houston; **Kevin W. Poindexter**, Katy, all of Tex.

[73] Assignee: **Shell Oil Company**, Houston, Tex.

[21] Appl. No.: 233,288

[22] Filed: Apr. 26, 1994

## Related U.S. Application Data

[63] Continuation of Ser. No. 108,785, Aug. 18, 1993, abandoned, which is a continuation of Ser. No. 842,858, Feb. 26, 1992, abandoned, which is a continuation-in-part of Ser. No. 764,272, Sep. 23, 1991, abandoned, and a continuation-in-part of Ser. No. 897,132, Jun. 11, 1992, abandoned, which is a continuation of Ser. No. 842,858, Feb. 26, 1992, abandoned, which is a continuation-in-part of Ser. No. 764,272, Sep. 23, 1991, abandoned.

[51] Int. Cl. 6 ..... C10L 1/22

[52] U.S. Cl. ..... 44/387; 44/415; 44/432

[58] Field of Search ..... 44/415, 432, 425, 44/387

## References Cited

### U.S. PATENT DOCUMENTS

4,038,044 7/1977 Garth .  
4,121,911 10/1978 Garth .  
4,160,648 7/1979 Lewis et al. .  
4,191,537 3/1980 Lewis et al. .  
4,197,409 4/1980 Lilburn .  
4,231,759 11/1980 Udelhofen et al. .

## FOREIGN PATENT DOCUMENTS

2010324 6/1979 United Kingdom .  
WO91/12303 8/1991 WIPO .

Primary Examiner—Margaret Medley

## ABSTRACT

Intake valve deposits in port fuel injected engines are reduced by using a fuel containing a mixture of (a) an oil soluble polyamine selected from (i) an aliphatic alkylene polyamine containing at least one olefinic polymer chain attached to a nitrogen and/or carbon atom of the alkylene radical(s) connecting the amino nitrogen atoms and said polyamine having a number average molecular weight in the range of from about 600 to about 10,000, (ii) a Mannich polyamine comprising the condensation product of a high molecular weight sulfur-free alkyl-substituted hydroxyaromatic compound wherein the alkyl group has a number average molecular weight from about 600 to about 10,000, an amine which contains an amino group having at least one active hydrogen atom, and an aldehyde, wherein the respective molar ratio of reactants is 1:0.1–10:0.1–10, or (iii) mixtures of (i) and (ii) and (b) an oil soluble hydrocarbyl poly(oxyalkylene)aminocarbamate having a number average molecular weight in the range of from about 600 to about 10,000 having at least one basic nitrogen atom wherein the hydrocarbyl group contains from 1 to about 30 carbons atoms, and wherein the mixture is present in an amount of 5–1000 ppmw basis the fuel and the weight ratio of component (a) to component (b) ranges from about 3:1 to about 1:2. The fuels are also compatible with carburetor and throttle body injected engines.

46 Claims, 1 Drawing Sheet





**GASOLINE COMPOSITION FOR REDUCING  
INTAKE VALVE DEPOSITS IN PORT FUEL  
INJECTED ENGINES**

This is a continuation of application Ser. No. 08/108,785, filed Aug. 18, 1993, now abandoned, which is a continuation of application Ser. No. 07/842,858, filed Feb. 26, 1992, now abandoned, which is a continuation-in-part of application Ser. No. 07/764,272, filed Sep. 23, 1991, now abandoned, and application Ser. No. 07/897,132 filed Jun. 11, 1992, now abandoned, which is a continuation of application Ser. No. 07/842,858 filed Feb. 26, 1992, now abandoned, which is a continuation-in-part of application Ser. No. 07/764,272 filed Sep. 23, 1991, now abandoned.

**BACKGROUND OF THE INVENTION**

1. Field of the Invention

The present invention relates to gasoline compositions for reducing intake valve deposits in port fuel injected engines.

2. Background

Gasoline compositions have traditionally been formulated to improve the performance of carburetor and throttle body injected engines. Beginning in about 1984, electronic port fuel injected engines were commonly introduced by automobile manufacturers. Shortly thereafter, in about 1985, problems began to be reported with intake valve deposits in electronic port fuel injected engines characterized by hard starting, stalls, and stumbles during acceleration and rough engine idle.

Accordingly, it would be desirable to have fuel compositions which reduced or eliminated such undesirable intake valve deposits in electronic port fuel injected engines. Also, since some carburetor and throttle body injector engines will still be in use for the foreseeable future, it would be desirable if such fuels could also be compatible with these engines. Intake valve detergency is generally defined by the BMW NA standard of intake valve cleanliness for unlimited mileage, which is an established correlation of good driveability with average intake valve deposit weight of 100 milligrams/valve or less.

Oil-soluble polyalkylene polyamines containing an olefinic polymer chain are known to improve detergent properties of fuels used in carburetor and throttle body type engines. These polyalkylene polyamines, particularly when used at high concentrations, can result in valve sticking and an increase in octane requirement. Various materials have been added to these polyalkylene polyamines to improve their performance. U.S. Pat. No. 5,006,130, issued April 9, 1991, discloses as a gasoline additive (a) polyalkylene polyamine and (b) at least one component selected from (i) a polymer of a C<sub>2</sub> to C<sub>6</sub> monoolefin, (ii) a copolymer of a C<sub>2</sub> to C<sub>6</sub> monoolefin, (iii) the corresponding hydrogenated polymer of copolymer, (iv) an oil soluble poly(oxyalkylene) alcohol, glycol or polyol or a mono or di ether thereof.

Hydrocarbylpoly(oxyalkylene)aminocarbamates have been disclosed in U.S. Pat. No. 4,197,409, issued Apr. 8, 1980 and U.S. Pat. No. 4,191,537, issued Mar. 4, 1980, as useful as deposit control additives which effectively control deposits in intake systems (carburetor, valves, etc.) of engines operated with fuels containing them, but which do not contribute to the combustion chamber deposits which cause increased octane requirements.

Mannich polyamines comprising the condensation product of a high molecular weight alkyl-substituted hydroxy aromatic compound, an amine which contains an amino

group having at least one active hydrogen atom, and an aldehyde have been disclosed in U.S. Pat. No. 4,231,759, issued Nov. 4, 1980, as useful for imparting detergency properties to an automotive fuel in order to keep intake valves clean.

**OBJECTS OF THE INVENTION**

It is an object of this invention to provide a gasoline additive combination which makes use of the good detergency properties of polyamines but which minimizes valve sticking and octane requirement increase which can result from the use of large amounts of polyamines.

It is further an object of this invention to provide a gasoline composition which reduces intake valve deposits in electronic port fuel injected engines and the poor driveability which is characteristic of intake valve deposition in these engines and which is also compatible with carburetor and throttle body injected engines which are still in use.

**SUMMARY OF THE INVENTION**

The present invention is directed to an unleaded gasoline composition comprising a major amount of a hydrocarbon base fuel of the gasoline boiling range containing an effective amount to reduce intake valve deposits in electronic port fuel injected engines of from about 5 ppmw to about 1000 ppmw based on the fuel composition of a mixture of (a) an oil soluble polyamine selected from the group consisting of (i) an aliphatic alkylene polyamine containing at least one olefinic polymer chain attached to a nitrogen and/or carbon atom of the alkylene radical(s) connecting the amino nitrogen atoms and said polyamine having a number average molecular weight in the range of from about 600 to about 10,000, (ii) a Mannich polyamine comprising the condensation product of a high molecular weight sulfur-free alkyl-substituted hydroxyaromatic compound wherein the alkyl group has a number average molecular weight from about 600 to about 3000, an amine which contains an amino group having at least one active hydrogen atom, and an aldehyde, wherein the respective molar ratio of reactants is 1:0.1-10:0.1-10, or (iii) mixtures of (i) and (ii) and (b) an oil soluble hydrocarbyl poly(oxyalkylene) aminocarbamate having a number average molecular weight in the range of from about 600 to about 10,000 having at least one basic nitrogen atom wherein said hydrocarbyl group contains from 1 to about 30 carbons atoms, and wherein the weight ratio of said polyamine to said hydrocarbyl poly(oxyalkylene) aminocarbamate ranges from about 3:1 to about 1:2.

**BRIEF DESCRIPTION OF THE DRAWING**

The sole drawing shows the synergistic improvement in intake valve deposit control obtained by using combinations of aliphatic alkylene polyamine and a hydrocarbyl poly(oxyalkylene) aminocarbamate.

**DESCRIPTION OF THE PREFERRED  
EMBODIMENTS**

Component (a)

Component (a) may be selected from either an aliphatic alkylene polyamine, a Mannich polyamine or mixtures of an aliphatic alkylene polyamine and a Mannich polyamine.

(i) Aliphatic Alkylene Polyamine

The oil soluble aliphatic alkylene polyamine component detergent (a) (i) has at least one polyester chain having an about 500 to about 9,900  $M_n$  (number average molecular

weight) and preferably from about 550 to about 4,900  $\overline{M}_n$ , and particularly from about 600 to about 1,300  $\overline{M}_n$ , and which may be saturated or unsaturated and straight or branched chain and attached to a nitrogen and/or carbon atom of the alkylene radicals connecting the amino-nitrogen atoms.

Preferred polyolefin-substituted polyalkylene polyamines have the structural formula I



where R is selected from the group consisting of a hydrogen atom and a polyolefin having a  $\overline{M}_n$  from about 500 to about 9,900, at least one R being a polyolefin group, R' is an alkylene radical having from 1 to 8 carbon atoms, preferably 1 to 4 carbon atoms, R'' is hydrogen or lower alkyl, and x is 0-5. Preferred is when one R is a branched-chain olefin polymer and the other R is hydrogen. The number average molecular weight range of R is preferably 550 to 4,900  $\overline{M}_n$ , with a range of 600-1300  $\overline{M}_n$  being particularly preferred.

The olefinic polymers (R) which are reacted with polyamines to form the additive of the present invention include olefinic polymers derived from alkanes or alkenes with straight or branched chains, which may or may not have aromatic or cycloaliphatic substituents, for instance, groups derived from polymers or copolymers of olefins which may or may not have a double bond. Examples of non-substituted alkenyl and alkyl groups are polyethylene groups, polypropylene groups, polybutylene groups, polyisobutylene groups, polyethylene-polypropylene groups, polyethylene-poly-alpha-methyl styrene groups and the corresponding groups without double bonds. Particularly preferred are polypropylene and especially polyisobutylene groups.

The R'' group may be hydrogen but is preferably lower alkyl, i.e., containing up to 7 carbon atoms, and more preferably is selected from methyl, ethyl, propyl and butyl groups.

The polyamines used to form the aliphatic polyamine compounds of this invention include primary and secondary low molecular weight aliphatic polyamines such as ethylene diamine, diethylene triamine, triethylene tetramine, propylene diamine, butylene diamine, trimethyl trimethylene diamine, tetramethylene diamine, diaminopentane or pentamethylene diamine, hexamethylene diamine, heptamethylene diamine, diaminooctane, decamethylene diamine, and higher homologues up to about 18 carbon atoms in the preparation of these compounds the same amines can be used or substituted amines can be used such as N-methyl ethylene diamine, N-propyl ethylene diamine, N,N-dimethyl 1,3-propane diamine, N-2-hydroxypropyl ethylene diamine, penta-(1-methylpropylene)hexamine, tetrabutylene-pentamine, hexa-(1,1-dimethylethylene)heptane, di-(1-methylamylene)-triamine, tetra-(1,3-dimethylpropylene)pentamine, penta-(1,5-dimethylamylene)-hexamine, di-(1-methyl-4-ethylbutylene)triamine, penta-(1,2-dimethyl-1-isopropylene)hexamine, tetraoctylenepentamine and the like.

Compounds possessing triamine as well as tetramine and pentamine groups are applicable for use because these can be prepared from technical mixtures of polyethylene polyamines, which could offer economic advantages.

The polyamine can be a cyclic polyamine, for instance, the cyclic polyamines formed when aliphatic polyamines with nitrogen atoms separated by ethylene groups were heated in the presence of hydrogen chloride.

An example of a suitable process for the preparation of the compounds employed according to the invention is the

reaction of a halogenated polyhydrocarbon having at least one halogen atom as a substituent and a hydrocarbon chain as defined hereinbefore for R with a polyamine. The halogen atoms are replaced by a polyamine group, while hydrogen halide is formed. The hydrogen halide can then be removed in any suitable way, for instance, as a salt with excess polyamine. The reaction between halogenated hydrocarbon and polyamine is preferably effected at elevated temperature in the presence of a solvent; particularly a solvent having a boiling point of at least about 160°C.

The reaction between polyhydrocarbon halide and a polyamine having more than one nitrogen atom available for this reaction is preferably effected in such a way that cross-linking is reduced to a minimum, for instance, by applying an excess of polyamine.

The amine additive according to the invention can be prepared, for example, by alkylation of low molecular weight aliphatic polyamines. For instance, a polyamine is reacted with an alkyl or alkenyl halide. The formation of the alkylated polyamine is accompanied by the formation of hydrogen halide, which is removed, for example, as a salt of starting polyamine present in excess. With this reaction between alkyl or alkenyl halide and the strongly basic polyamines, dehalogenation of the alkyl or alkenyl halide can occur as a side reaction, so that hydrocarbons are formed as by-products. Their removal can, without objection, be omitted.

The number average molecular weight of the aliphatic alkylene polyamine will range from about 600 to about 10,000  $\overline{M}_n$ , preferably from about 600 to about 5000  $\overline{M}_n$ , and most preferably from about 600 to about 1500  $\overline{M}_n$ .

#### (ii) Mannich Polyamine

The oil soluble Mannich polyamine component detergent (a) (ii) comprises a condensation product of a high molecular weight alkyl-substituted hydroxyaromatic compound, an amine which contains an amino group having at least one active hydrogen atom (preferably a polyamine), and an aldehyde. Such condensation products can be prepared by condensing in the usual manner under Mannich reaction conditions:

- (1) an alkyl-substituted hydroxyaromatic compound, whose alkyl-substituent has a 600-10,000  $\overline{M}_n$ , preferably a polyalkylphenol whose polyalkyl substituent is derived from 1-mono-olefin polymers having a  $\overline{M}_n$  of about 600-3,000, more preferably about 750-1200, and most preferably 1000-1100;
- (2) an amine (preferably a polyamine) containing at least one  $\text{NH}$  group, preferably an alkylene polyamine of the formula



wherein A is a divalent alkylene radical having 2 to 6 carbon atoms and x is an integer from 1 to 10; and

- (3) an aldehyde, preferably formaldehyde.

The Mannich polyamine utilized is described in detail in U.S. Pat. No. 4,231,759, issued Nov. 4, 1980, which is incorporated by reference herein. The foregoing high molecular weight products employed in the fuels of this invention are preferably prepared according to the conventional methods heretofore employed for the preparation of Mannich condensation products, using the above-named reactants in the respective molar ratios of high molecular weight alkyl-substituted hydroxyaromatic compound, amine and aldehyde of approximately 1:0.1-10:0.1-10. A suitable

condensation procedure involves adding at a temperature of from room temperature to about 93° C. the formaldehyde reagent (e.g. Formalin) to a mixture of reagents (1) and (2) above alone or in an easily removed organic solvent, such as benzene, xylene or toluene or in solvent-refined neutral oil and then heating the reaction mixture to an elevated temperature (120°–175° C.) while preferably blowing with an inert stripping gas, such as nitrogen, carbon dioxide, etc. until dehydration is complete. The product so obtained is finished by filtration and dilution as desired.

The preferred detergent additives employed in this invention are high molecular weight Mannich condensation products, formed by reacting (1) an alkylphenol, whose alkyl group has 600–3,000 Mn; (2) an ethylene polyamine, an amine reactant; and (3) a formaldehyde affording reactant in the respective molar ratio of 1.0:0.5–2.0:1.0–3.0.

Representative of the high molecular weight alkyl-substituted hydroxyaromatic compounds are polypropylphenol, polybutylphenol and other polyalkylphenols. These polyalkylphenols may be obtained by the alkylation, in the presence of an alkylating catalyst; such as  $\text{BF}_3$ , of phenol with high molecular weight polypropylene, polybutylene and other polyalkylene compounds to give alkyl substituents on the benzene ring of phenol having an average 600–100, 000 Mn.

The 600 Mn and higher Mn alkyl-substituents on the hydroxyaromatic compounds may be derived from high molecular weight polypropylenes, polybutenes and other polymers of mono-olefins, principally 1-monoolefins. Also useful are copolymers of mono-olefins with monomers copolymerizable therewith wherein the copolymer molecular contains at least 90%, by weight, of mono-olefin units. Specific examples are copolymers of butenes (butene-1, butene-2 and isobutylene) with monomers copolymerizable therewith wherein the copolymer contains at least 90% by weight, of propylene and butene units, respectively. Said monomers copolymerizable with propylene or said butenes include monomers containing a small proportion of unreactive polar groups such as chloro, bromo, keto, ether, aldehyde, which do appreciably lower the oil-solubility of the polymer. The comonomers polymerized with propylene or said butenes may be aliphatic and can also contain non-aliphatic groups, e.g., styrene, methylstyrene, p-dimethylstyrene, divinyl benzene and the like. From the foregoing limitation placed on the monomer copolymerized with propylene or said butenes, it is abundantly clear that said polymers and copolymers of propylene and said butenes are substantially aliphatic hydrocarbon polymers. Thus the resulting alkylated phenols contain substantially alkyl hydrocarbon substituents having Mn upward from 600.

In addition to these high molecular weight hydroxyaromatic compounds others which may be used include, exclusive of sulfurized derivatives, high molecular weight alkyl-substituted derivatives of resorcinol, hydroquinone, cresol, catechol, xylanol, hydroxy diphenyl, benzylphenol, phenethylphenol, naphthol, tolynaphthol, among others. Preferred for the preparation of such preferred Mannich condensation products are the polyalkylphenol reactants, e.g., polypropylphenol and polybutylphenol whose alkyl group has a 600–3,000 Mn, the more preferred alkyl groups having a 740–1,200 Mn, while the most preferred alkyl groups is a polypropyl group having a 800–850 Mn, desirably about 825 Mn.

The preferred configuration of the alkyl-substituted hydroxyaromatic compound is that of a para-substituted mono-alkylphenol. However, any alkylphenol readily reactive in the Mannich condensation reaction may be

employed. Accordingly, ortho mono-alkylphenols and dialkylphenols are suitable for use in this invention.

Various amine reactants may be utilized including mono and polyamines. The preferred amine reactants are alkylene polyamines, principally polyethylene polyamines. Other representative organic compounds containing at least one  $\text{HN}^+$  group suitable for use in the preparation of Mannich condensation products are well known and include the mono and di-amino alkanes and their substituted analogs, e.g., ethylamine, dimethylamine, dimethylaminopropyl amine and diethanol amine; aromatic diamines, e.g., phenylene diamine, diamino naphthalenes; heterocyclic amines, e.g., morpholine, pyrrole, pyrroldine, imidazole, imidazolidine, and piperidine; melamine and their substituted analogs.

Suitable alkylene polyamine reactants include ethylenediamine, diethylene triamine, triethylene tetramine, tetraethylene pentamine, pentaethylene hexamine, hexaethylene heptamine, heptaethylene octamine, octaethylene nonamine, nonaethylene decamine, decaethylene undecamine and mixtures of such amines having nitrogen contents corresponding to the alkylene polyamines, in the formula  $\text{H}_2\text{N}^+-(\text{A}-\text{NH}-)^n\text{H}$ , mentioned before, where A is divalent ethylene and n is an integer from 1 to 10. Corresponding propylene polyamines such as propylene diamine and di-, tri-, tetra-, penta-propylene tri-, tetra-, penta- and hexa-amines are also suitable reactants. The alkylene polyamines are usually obtained by the reaction of ammonia and dihalo alkanes, such as dichloro alkanes. Thus the alkylene polyamines obtained from the reaction of 2 to 11 moles of ammonia with 1 to 10 moles of dichloro alkanes having 2 to 6 carbon atoms and the chlorines on different carbons are suitable alkylene polyamine reactants.

Representative aldehydes for use in the preparation of the high molecular products of this invention include the aliphatic aldehydes such as formaldehyde (including paraformaldehyde and Formalin), acetaldehyde and aldol (b-hydroxybutyraldehyde). We prefer to use formaldehyde or a formaldehydielding reactant.

(iii) Mixtures of the Aliphatic Alkylene Polyamine and the Mannich Polyamine

Mixtures of components (a)(i) and (a)(ii) may also be suitably combined with component (b) to prepare the additive composition used in the present invention.

#### Component (b)—Aminocarbamate

The amine moiety of the hydrocarbyl-terminated poly(oxyalkylene) aminocarbamate is preferably derived from a polyamine having from 2 to about 12 amine nitrogen atoms and from 2 to about 40 carbon atoms. The polyamine is preferably reacted with a hydrocarbyl poly(oxyalkylene) chloroformate to produce the hydrocarbyl poly(oxyalkylene) aminocarbamate fuel additive component (b). The chloroformate is itself derived from hydrocarbyl poly(oxyalkylene) alcohol by reaction with phosgene. The polyamine, encompassing diamines, provides the product poly(oxyalkylene) aminocarbamate with, on the average, at least about one basic nitrogen atom per carbamate molecule, i.e., a nitrogen atom titratable by strong acid. The polyamine preferably has a carbon-to-nitrogen ratio of from about 1:1 to about 10:1. The polyamine may be substituted with substituents selected from hydrogen, hydrocarbyl groups of from 1 to about 10 carbon atoms, acyl groups of from 2 to about 10 carbon atoms, and monoketone, mono-hydroxy, mononitro, monocyno, alkyl and alkoxy derivatives of hydrocarbyl groups of from 1 to 10 carbon atoms. It is preferred that at least one of the basic nitrogen atoms of the polyamine is a primary or secondary amino nitrogen. The polyamine component has been described and exem-

plified more fully in U.S. Pat. No. 4,191,537, issued Mar. 4, 1980, incorporated by reference herein.

Hydrocarbyl, as used in describing all the components of this invention, denotes an organic radical composed of carbon and hydrogen which may be aliphatic, alicyclic, aromatic or combination thereof, e.g., aralkyl. Preferably, the hydrocarbyl group will be relatively free of aliphatic unsaturation, i.e., ethylenic and acetylenic, particularly acetylenic unsaturation. The more preferred polyamine for the aminocarbamate component is a polyalkylene polyamine, including alkylenediamine, and including substituted polyamines, e.g., alkyl and hydroxylalkyl-substituted polyalkylene polyamine. Preferably, the alkylene group contains from 2 to 6 carbon atoms, there being preferably from 2 to 3 carbon atoms between the nitrogen atoms. Examples of such polyamines include ethylenediamine, diethylene triamine, triethylene tetramine, di(trimethylene)triamine, dipropylene triamine, tetraethylene pentamine, etc. Among the polyalkylene polyamines are polyethylene polyamine, polypropylene polyamine containing 2-12 amine nitrogen atoms and 2-24 carbon atoms are especially preferred and in particular, the lower polyalkylene polyamines, e.g., ethylenediamine, dipropylene triamine, etc., are most preferred.

The hydrocarbyl-terminated poly(oxyalkylene) polymers which are utilized in preparing the aminocarbamates are monohydroxy compounds, e.g., alcohols, often termed monohydroxy polyethers, or polyalkylene glycol monocarbonyl ethers, or "capped" poly(oxyalkylene) glycols, and are to be distinguished from the poly(oxyalkylene) glycols (diols), or polyols, which are not hydrocarbyl-terminated, i.e., are not capped. The hydrocarbyl-terminated poly(oxyalkylene) alcohols are produced by the addition of lower alkylene oxides, such as ethylene oxide, propylene oxide, butylene oxide, etc. to the hydroxy compound ROH under polymerization conditions, wherein R is the hydrocarbyl group which caps the poly(oxyalkylene) chain. In the poly(oxyalkylene) component of the aminocarbamate, the group R will generally contain from 1 to about 30 carbon atoms, preferably from 2 to about 20 carbon atoms and is preferably aliphatic or aromatic, i.e., an alkyl or alkyl phenyl wherein the alkyl is a straight or branched-chain of from 1 to about 24 carbon atoms. The oxyalkylene units in the poly(oxyalkylene) component preferably contain from 2 to about 5 carbon atoms but one or more units of a larger carbon number may also be present. Each poly(oxyalkylene) polymer contains at least about 5 oxyalkylene units, preferably 8 to about 100 oxyalkylene units, more preferably about 10-100 units and most preferably 10 to about 25 such units. The poly(oxyalkylene) component is more fully described and exemplified in U.S. Pat. Nos. 4,191,537, issued Mar. 4, 1980, and 4,197,409, issued Apr. 8, 1980, incorporated by reference herein. The poly(oxyalkylene) aminocarbamate fuel additive used in compositions of the present invention is obtained by linking the amine component and the poly(oxyalkylene) component together through a carbamate linkage, i.e.,



wherein the oxygen may be regarded as the terminal hydroxyl oxygen of the poly(oxyalkylene) alcohol component, and the carbonyl group,  $-\text{C}(\text{O})-$ , is preferably provided by a coupling agent, e.g., phosgene. In the preferred method of preparation the hydrocarbyl poly(oxyalkylene) alcohol is reacted with phosgene to produce a chloroformate and the chloroformate is reacted with the polyamine. The carbamate linkages are formed as the poly(oxyalkylene)

chains are bound to the nitrogen of the polyamine to the oxycarbonyl group of the chloroformate. Since there may be more than one nitrogen atom of the polyamine which is capable of reacting with the chloroformate, the aminocarbamate contains at least one hydrocarbyl poly(oxyalkylene) polymer chain bonded through an oxycarbonyl group to a nitrogen atom of the polyamine, but the carbonate may contain from 1 to 2 or more such chains. It is preferred that the hydrocarbyl poly(oxyalkylene) aminocarbamate product contains, on the average, about 1 poly(oxyalkylene) chain per molecule (i.e., is a monocarbamate), although it is understood that this reaction route may lead to mixtures containing appreciable amount of di- or higher poly(oxyalkylene) chain substitution on a polyamine containing several reactive nitrogen atoms. Several especially preferred aminocarbamates are butyl-poly(oxyalkylene)-N-(2-aminoethyl) carbamate and alkylphenyl-poly(oxyalkylene)-N-(2-aminoethyl) carbamate. A particularly preferred carbamate can be expressed by the following formula:



wherein R is hydrogen, alkyl and "n" preferably is greater than about 5. Aminocarbamates suitable for use in the instant invention can be obtained from the Oronite Additives Division of Chevron Chemical Company.

Synthetic methods to avoid higher degrees of substitution, methods of preparation, and other characteristics of the aminocarbamate used as component (b) are more fully described and exemplified in the above-mentioned U.S. Pat. Nos. 4,191,537 and 4,197,409.

The number average molecular weight of the aminocarbamate will range from about 600 to about 10,000  $\bar{M}_n$ , preferably from about 600 to about 5000  $\bar{M}_n$  and most preferably from about 600 to about 2000  $\bar{M}_n$ .

The total amounts of component (a) and component (b) present in the fuel composition will range from about 5 to about 1000, preferably from about 50 to about 1000, more preferably from about 50 to about 500 and even more preferably from about 100 to about 400 and most preferably from about 200 to about 300 parts per million by weight (ppmw) based on the fuel composition. In particularly preferred embodiments, the total amounts of component (a) and component (b) present in the fuel composition will be about 200 part per million weight (ppmw) or about 250 parts per million weight (ppmw) based on the fuel composition. The weight ratio, component (a): component (b), will range from about 3:1 to about 1:2 and preferably from about 2:1 to about 2:3. In a particularly preferred embodiment the weight ratio is set at about 1:1.

Suitable liquid hydrocarbon fuels of the gasoline boiling range are mixtures of hydrocarbons having a boiling range of from about 25° C. to about 232° C. and comprise mixtures of saturated hydrocarbons, olefinic hydrocarbons and aromatic hydrocarbons. Preferred are gasoline blends having a saturated hydrocarbon content ranging from about 40 to about 80 percent volume, an olefinic hydrocarbon content from about 0 to about 30 percent volume and an aromatic hydrocarbon content ranging from about 10 to about 60 percent volume. The base fuel can be derived from straight run gasoline, polymer gasoline, natural gasoline, dimer or trimerized olefins, synthetically produced aromatic hydrocarbon mixtures from thermally or catalytically reformed hydrocarbons, or from catalytically cracked or thermally cracked petroleum stocks, and the like or mixtures of these.

The hydrocarbon composition and octane level of the base fuel are not critical. The octane level, (R+M)/2, will generally be above 85. Any conventional motor fuel base may be employed in the practice of this invention. For example, in the gasoline, hydrocarbons can be replaced by up to substantial amounts of conventional alcohols, or ethers, conventionally known for use in fuels. The base fuels are desirably substantially free of water, since water could impede a smooth combustion.

Normally, the hydrocarbon fuel mixtures to which the invention is applied are essentially lead-free, but can contain minor amounts of blending agents such as methanol, ethanol, methyl tertiary butyl ether, and the like, e.g., at from about 0.1 to about 15% volume of the base fuel. The fuels can also contain antioxidants such as phenolics, e.g., 2,6-di-tert-butylphenol or phenylenediamines, e.g., N,N'-di-sec-butyl-p-phenylenediamine, dyes, metal deactivators, dehazers such as polyester-type ethoxylated alkylphenol-formaldehyde resins and the like. Corrosion inhibitors, such as a polyhydric alcohol ester of a succinic acid derivative having on at least one of its alpha-carbon atoms an unsubstituted or substituted aliphatic hydrocarbon group having 20 to 500 carbon atoms, for example, pentaerythritol diester of polyisobutylene-substituted succinic acid, the polyisobutylene group having a number average molecular weight of about 950, in an amount of about 1 to 1000 ppmw. The fuels may also contain antiknock compounds such as a methyl cyclopentadienylmanganese tricarbonyl, ortho-azio-phenol and the like as well as co-antiknock compounds such as benzoylacetone.

The additives of the present invention can be added to the fuel neat or in the form of a concentrate. For example, the agent can be added separately to the fuel or blended with the other fuel additives. A concentrate can be prepared comprising a major amount of the additive mixture of the invention and a minor amount of a fuel compatible diluent boiling in the range of about 50° C. to 232° C. The additive can be added to the fuel at any point prior to its delivery to the end user.

The invention also provides a method for operating a port fuel injected engine on an unleaded fuel compatible with carburetor and throttle body injected engines which comprises introducing into an electronic port fuel injected engine with the combustion intake charge an effective amount of a mixture of (a) an oil soluble polyamine selected from the group consisting of (i) an aliphatic alkylene polyamine, (ii) a Mannich amine, or (iii) mixtures of (i) and (ii) and (b) an oil soluble hydrocarbyl poly(oxyalkylene) aminocarbamate in the before-described amounts and ratios.

The ranges and limitations provided in the instant specification and claims are those which are believed to particularly point out and distinctly claim the instant invention. It is, however, understood that other ranges and limitations that perform substantially the same function in substantially the same way to obtain the same or substantially the same result are intended to be within the scope of the instant invention as defined by the instant specification and claims.

The invention will be described by the following examples which are provided for illustrative purposes and are not to be construed as limiting the invention.

#### Illustrative Embodiment I

This example illustrates the beneficial effect on intake valve deposits of a gasoline additive comprising a mixture of an aliphatic alkylene polyamine and a hydrocarbyl poly(oxyalkylene) aminocarbamate.

Intake valve deposit tests were conducted in a BMW 325 car equipped with the 2.7-liter, six-cylinder engine with port fuel injection, and was operated for 8,050 kilometers on the test fuel. Before the test started, deposits were removed from the cylinder head, intake manifold and piston tops and new intake valves were weighed and installed. The oil and filter were changed, new spark plugs installed and the fuel injectors flow checked. Mileage was accumulated on a road simulation dynamometer. A four minute test cycle was employed. It consisted of a 2 minute acceleration from 54 to 75 km/hr, a 1 minute acceleration to 112 km/hr and a 1 minute deceleration to 54 km/hr. The average speed was about 79 km/hr and the cycle was repeated until 8050 kilometers were accumulated (about 102 hrs).

Table 1 lists the additive compositions used in premium unleaded base gasolines and the average (of six) intake valve deposit weights at the end of the test (8,050 kilometers).

TABLE 1

| Com-<br>position | Component<br>(a)(i) <sup>1</sup><br>ppmw | Component<br>(b) <sup>2</sup><br>ppmw | Ratio<br>(a)/(b) | BMW 325 Results<br>Avg. Deposit<br>weight, mg |
|------------------|------------------------------------------|---------------------------------------|------------------|-----------------------------------------------|
| 1                | 200                                      | 0                                     | 200:0            | 39.0                                          |
| 2                | 150                                      | 50                                    | 3:1              | 34.3                                          |
| 3                | 100                                      | 100                                   | 1:1              | 34.6                                          |
| 4                | 50                                       | 150                                   | 1:3              | 148.6                                         |
| 5                | 0                                        | 200                                   | 0:200            | 153.6                                         |

<sup>1</sup>Component (a)(i) is H-polyisobutetyl-N,N'-dimethyl-1,3-diaminopropane. Mn = 1050.

<sup>2</sup>Component (b) is a hydrocarbyl poly(oxyalkylene) aminocarbamate obtained from the Oronite Additives Division of Chevron Chemical Company as OGA 480. Mn = 1400-1800.

Results of these tests are also plotted in the Figure and demonstrate that the gasoline compositions of the invention provide a synergistic improvement in intake valve deposit reduction while concomitantly allowing for the reduction in the amount of aliphatic alkylene polyamine thereby lessening the known effect of the polyamine to cause valve sticking.

#### Illustrative Embodiment II

Intake valve deposit tests were conducted in a BMW 318i car equipped with the 1.8-liter, four-cylinder engine which was operated for 10,000 miles on the test fuel. Before the test started, deposits were removed from the cylinder head, intake manifold and piston tops and new intake valves were weighed and installed. The oil and filter were changed, new spark plugs installed and the fuel injectors flow checked. Mileage was accumulated on public roads using trained drivers. The test route consisted of about 10% city driving, 20% on secondary roads and 70% highway driving (maximum speed of 65 mph).

The primary test data was the intake valve deposit (IVD) weights at the end of the 10,000-mile test. BMW's pass criteria are as follows: an average deposit weight of 100 milligrams/valve or less at the conclusion of the test meets BMW requirements for unlimited mileage acceptance; an average deposit weight of 250 mg/valve or less at the conclusion of the test meets BMW's requirement for 50,000-mile service.

Table 2 lists the additive compositions used in regular unleaded base gasolines and the average intake valve deposit weights at the end of the test (10,000 miles).

TABLE 2

| Com-<br>position | Component<br>(a)<br>ppmw | Component<br>(b)<br>ppmw | Ratio<br>(a)/(b) | BMW 318i Results<br>Avg. Deposit<br>weight, mg |
|------------------|--------------------------|--------------------------|------------------|------------------------------------------------|
| 1                | 125 <sup>1</sup>         | 125 <sup>2</sup>         | 1:1              | 0                                              |
| 2                | 125 <sup>3</sup>         | 125 <sup>2</sup>         | 1:1              | 44                                             |

<sup>1</sup>Component (a) is the Amoco Mannich Amine known as "Amoco 596" described in U.S. Pat. No. 4,231,759. Mn = 1000-1100.

<sup>2</sup>Component (b) is a hydrocarbyl poly(oxyalkylene) aminocarbamate, Mn = 1400-1800, obtained from the Oronite Additives Division of Chevron Chemical Company as OGA 480.

<sup>3</sup>Component (a) is N-polyisobutlenyl-N',N'-dimethyl-1,3-diaminopropane. Mn = 1050

Comparing the values of intake valve deposits in Table 2 with the similar values in Table 1 (at a ratio of (a)/(b) of 1:1) it can be seen that the aliphatic alkylene polyamines of Table 1 can be replaced with the Mannich polyamine of Table 2 with substantially the same results.

What is claimed is:

1. An unleaded fuel composition comprising a major amount of a hydrocarbon base fuel of the gasoline boiling range containing an effective amount to reduce intake valve deposits in electronic port fuel injected engines of from about 50 ppmw to about 500 ppmw based on the fuel composition of a mixture of (a) an oil soluble polyamine selected from the group consisting of (i) an aliphatic alkylene polyamine containing at least one olefinic polymer chain attached to a nitrogen and/or carbon atom of the alkylene radical(s) connecting the amino nitrogen atoms, said alkylene group having from 1 to 8 carbon atoms, and said polyamine having a number average molecular weight in the range of from about 600 to about 10,000, (ii) a Mannich polyamine comprising the condensation product of a high molecular weight sulfur-free alkyl-substituted hydroxyaromatic compound wherein the alkyl group has a number average molecular weight from about 600 to about 10,000, an amine which contains an amino group having at least one active hydrogen atom, and an aldehyde, wherein the respective molar ratio of reactants is 1:0.1-10:0.1-10, or (iii) mixtures of (i) and (ii) and (b) an oil soluble hydrocarbyl poly(oxyalkylene) aminocarbamate having a number average molecular weight in the range of from about 600 to about 10,000 having at least one basic nitrogen atom and from about 10 to about 100 oxyalkylene groups wherein said hydrocarbyl group contains from 1 to about 30 carbon atoms, said oxyalkylene groups contain from about 2 to about 5 carbon atoms and wherein the weight ratio of said polyamine to said hydrocarbyl poly(oxyalkylene)aminocarbamate ranges from about 3:1 to about 1:2.

2. The composition of claim 1 wherein the aliphatic alkylene polyamine has a number average molecular weight in the range of from about 600 to about 5000, the alkyl group of the Mannich polyamine has a number average molecular weight in the range of from about 600 to about 3,000, and the aminocarbamate has a number average molecular weight in the range of from about 600 to about 5000.

3. The composition of claim 2 wherein the aliphatic alkylene polyamine has a number average molecular weight in the range of from about 600 to about 1500, the alkyl group of the Mannich polyamine has a number average molecular weight in the range of from about 1000 to about 1100, and the aminocarbamate has a number average molecular weight in the range of from about 600 to about 2000.

4. The composition of claim 1 wherein weight of the mixture of polyamine and aminocarbamate ranges from about 100 ppmw to about 400 ppmw based on the fuel composition.

5. The composition of claim 4 wherein the weight of the mixture of polyamine and aminocarbamate ranges from about 200 ppmw to about 300 ppmw based on the fuel composition.

6. The composition of claim 4 wherein the weight ratio of polyamine to aminocarbamate ranges from about 2:1 to about 2:3.

7. The composition of claim 4 wherein the weight ratio of polyamine to aminocarbamate is about 1:1.

8. The fuel composition of claim 4 wherein the oil soluble polyamine is an aliphatic alkylene polyamine.

9. The fuel composition of claim 4 wherein the oil soluble polyamine is a Mannich polyamine.

10. The composition of claim 5 wherein the weight ratio of polyamine to aminocarbamate ranges from about 2:1 to about 2:3.

11. The composition of claim 5 wherein the weight ratio of polyamine to aminocarbamate is about 1:1.

12. A method for operating an electronic port fuel injected engine on an unleaded fuel composition compatible with carburetor and throttle body injected engines which comprises introducing into an electronic port fuel injected engine with the combustion intake charge an amount of from about 50 ppmw to about 500 ppmw to reduce intake valve deposits

15 of a mixture of (a) an oil soluble polyamine selected from the group consisting of (i) an aliphatic alkylene polyamine containing at least one olefinic polymer chain attached to a nitrogen and/or carbon atom of the alkylene radical(s) connecting the amino nitrogen atoms, said alkylene group having from 1 to 8 carbon atoms, and said polyamine having

20 a number average molecular weight in the range of from about 600 to about 10,000, (ii) a Mannich polyamine comprising the condensation product of a high molecular weight sulfur-free alkyl-substituted hydroxyaromatic compound

25 wherein the alkyl group has a number average molecular weight from about 600 to about 10,000, an amine which contains an amino group having at least one active hydrogen atom, and an aldehyde, wherein the respective molar ratio of reactants is 1:0.1-10:0.1-10, or (iii) mixtures of (i) and (ii)

30 and (b) an oil soluble hydrocarbyl poly(oxyalkylene)aminocarbamate having a number average molecular weight in the range of from about 600 to about 10,000 having at least one basic nitrogen atom and from about 10 to about 100 oxyalkylene groups wherein said hydrocarbyl group contains from 1 to about 30 carbon atoms, said oxyalkylene groups contain from about 2 to about 5 carbon atoms and wherein the weight ratio of said polyamine to said hydrocarbyl poly(oxyalkylene)aminocarbamate ranges from

35 about 3:1 to about 1:2.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8

16. The method of claim 15 wherein the weight of the mixture of polyamine and aminocarbamate ranges from about 200 ppmw to about 300 ppmw based on the fuel composition.

17. The method of claim 15 wherein the weight ratio of polyamine to aminocarbamate ranges from about 2:1 to about 2:3.

18. The method of claim 15 wherein the weight ratio of polyamine to aminocarbamate is about 1:1.

19. The method of claim 15 wherein the oil soluble polyamine is an aliphatic alkylene polyamine.

20. The method of claim 15 wherein the oil soluble polyamine is a Mannich polyamine.

21. The method of claim 16 wherein the weight ratio of polyamine to aminocarbamate ranges from about 2:1 to about 2:3.

22. The method of claim 16 wherein the weight ratio of polyamine to aminocarbamate is about 1:1.

23. An unleaded fuel composition comprising a major amount of a hydrocarbon base fuel of the gasoline boiling range containing an effective amount to reduce intake valve deposits in electronic port fuel injected engines of about 250 ppmw based on the fuel composition of a mixture of (a) an oil soluble polyamine selected from the group consisting of (i) an aliphatic alkylene polyamine containing at least one olefinic polymer chain attached to a nitrogen and/or carbon atom of the alkylene radical(s) connecting the amino nitrogen atoms, said alkylene group having from 1 to 8 carbon atoms, and said polyamine having a number average molecular weight in the range of from about 600 to about 10,000, (ii) a Mannich polyamine comprising the condensation product of a high molecular weight sulfur-free alkyl-substituted hydroxyaromatic compound wherein the alkyl group has a number average molecular weight from about 600 to about 10,000, an amine which contains an amino group having at least one active hydrogen atom, and an aldehyde, wherein the respective molar ratio of reactants is 1:0.1-10:0.1-10, or (iii) mixtures of (i) and (ii) and (b) an oil soluble hydrocarbyl poly(oxyalkylene)aminocarbamate having a number average molecular weight in the range of from about 600 to about 10,000 having at least one basic nitrogen atom and from about 10 to about 100 oxyalkylene groups wherein said hydrocarbyl group contains from 1 to about 30 carbons atoms, said oxyalkylene groups contain from about 2 to about 5 carbon atoms and wherein the weight ratio of said polyamine to said hydrocarbyl poly(oxyalkylene)aminocarbamate is about 1:1.

24. A method for operating an electronic port fuel injected engine on an unleaded fuel composition compatible with carburetor and throttle body injected engines which comprises introducing into an electronic port fuel injected engine with the combustion intake charge an amount of about 250 ppmw to reduce intake valve deposits of a mixture of (a) an oil soluble polyamine selected from the group consisting of (i) an aliphatic alkylene polyamine containing at least one olefinic polymer chain attached to a nitrogen and/or carbon atom of the alkylene radical(s) connecting the amino nitrogen atoms, said alkylene group having from 1 to 8 carbon atoms, and said polyamine having a number average molecular weight in the range of from about 600 to about 10,000, (ii) a Mannich polyamine comprising the condensation product of a high molecular weight sulfur-free alkyl-substituted hydroxyaromatic compound wherein the alkyl group has a number average molecular weight from about 600 to about 10,000, an amine which contains an amino group having at least one active hydrogen atom, and an aldehyde, wherein the respective molar ratio of reactants is

1:0.1-10:0.1-10, or (iii) mixtures of (i) and (ii) and (b) an oil soluble hydrocarbyl poly(oxyalkylene)aminocarbamate having a number average molecular weight in the range of from about 600 to about 10,000 having at least one basic nitrogen atom and from about 10 to about 100 oxyalkylene groups wherein said hydrocarbyl group contains from 1 to about 30 carbons atoms, said oxyalkylene groups contain from about 2 to about 5 carbon atoms and wherein the weight ratio of said polyamine to said hydrocarbyl poly(oxyalkylene)aminocarbamate is about 1:1.

25. An unleaded fuel composition comprising a major amount of a hydrocarbon base fuel of the gasoline boiling range containing an effective amount to reduce intake valve deposits in electronic port fuel injected engines of from about 100 ppmw to about 400 ppmw based on the fuel composition of a mixture of (a) an oil soluble aliphatic alkylene polyamine containing at least one olefinic polymer chain attached to a nitrogen and/or carbon atom of the alkylene radical(s) connecting the amino nitrogen atoms, said alkylene group having from one to four carbon atoms, and said polyamine having a number average molecular weight in the range of from about 600 to about 1,500 and (b) an oil soluble hydrocarbyl poly(oxyalkylene)aminocarbamate having a number average molecular weight in the range of from about 600 to about 2,000 having at least one basic nitrogen atom and from about 10 to about 25 oxyalkylene groups wherein said hydrocarbyl group contains from 1 to about 30 carbons atoms, said oxyalkylene groups contain from about 2 to about 5 carbon atoms and wherein the weight ratio of said aliphatic alkylene polyamine to said hydrocarbyl poly(oxyalkylene)aminocarbamate ranges from about 3:1 to about 1:2.

26. The composition of claim 25 wherein the weight of the mixture of polyamine and aminocarbamate ranges from about 200 ppmw to about 300 ppmw based on the fuel composition.

27. The composition of claim 26 wherein the aliphatic alkylene polyamine has a number average molecular weight of about 1050 and the hydrocarbyl poly(oxyalkylene)aminocarbamate has a number average molecular weight of from about 1400 to about 1800.

28. The composition of claim 26 wherein the weight ratio of said aliphatic alkylene polyamine to said hydrocarbyl poly(oxyalkylene)aminocarbamate is about 1:1.

29. The composition of claim 28 wherein the aminocarbamate is alkylphenyl-poly(oxyalkylene)-N-(2-aminoethyl)carbamate.

30. A method for operating an electronic port fuel injected engine on an unleaded fuel composition compatible with carburetor and throttle body injected engines which comprises introducing into an electronic port fuel injected engine with the combustion intake charge an effective amount of from about 100 ppmw to about 400 ppmw to reduce intake valve deposits of a mixture of (a) an oil soluble aliphatic alkylene polyamine selected from the group consisting of (i) an aliphatic alkylene polyamine containing at least one olefinic polymer chain attached to a nitrogen and/or carbon atom of the alkylene radical(s) connecting the amino nitrogen atoms, said alkylene group having from one to four carbon atoms, and said polyamine having a number average molecular weight in the range of from about 600 to about 1,500 and (b) an oil soluble hydrocarbyl poly(oxyalkylene)aminocarbamate having a number average molecular weight in the range of from about 600 to about 2,000 having at least one basic nitrogen atom and from about 10 to about 25 oxyalkylene groups wherein said hydrocarbyl group contains from 1 to about 30 carbons atoms, said oxyalkylene

groups contain from about 2 to about 5 carbon atoms and wherein the weight ratio of said aliphatic alkylene polyamine to said hydrocarbyl poly(oxyalkylene)aminocarbamate ranges from about 3:1 to about 1:2.

31. The method of claim 30 wherein the weight of the mixture of polyamine and aminocarbamate ranges from about 200 ppmw to about 300 ppmw based on the fuel composition.

32. The method of claim 31 wherein the aliphatic alkylene polyamine has a number average molecular weight of about 1050 and the hydrocarbyl poly(oxyalkylene)aminocarbamate has a number average molecular weight of about 1400 to about 1800.

33. The method of claim 32 wherein the weight ratio of said aliphatic alkylene polyamine to said hydrocarbyl poly(oxyalkylene)aminocarbamate is about 1:1.

34. The method of claim 31 wherein the aminocarbamate is alkylphenyl-poly(oxyalkylene)-N-(2-aminoethyl)carbamate.

35. An unleaded fuel composition comprising a major amount of a hydrocarbon base fuel of the gasoline boiling range containing an effective amount to reduce intake valve deposits in electronic port fuel injected engines of from about 200 ppmw to about 300 ppmw based on the fuel composition of a mixture of (a) a N-polyisobutetyl-N',N'-dimethyl-1,3-diaminopropane having a number average molecular weight in the range of from about 600 to about 1500 and (b) an alkylphenyl-poly(oxyalkylene)-N-(2-aminoethyl)carbamate having a number average molecular weight in the range of from about 1400 to about 1800 having at least one basic nitrogen atom and from about 10 to about 25 oxyalkylene groups wherein said alkylphenyl group contains from 1 to about 30 carbons atoms, said oxyalkylene groups contain from about 2 to about 5 carbon atoms and wherein the weight ratio of said N-polyisobutetyl-N',N'-dimethyl-1,3-diaminopropane to said alkylphenyl-poly(oxyalkylene)-N-(2-aminoethyl)carbamate ranges from about 3:1 to about 1:2.

36. A method for operating an electronic port fuel injected engine on an unleaded fuel composition compatible with carburetor and throttle body injected engines which comprises introducing into an electronic port fuel injected engine with the combustion intake charge an effective amount of from about 200 ppmw to about 300 ppmw to reduce intake valve deposits of a mixture of (a) a N-polyisobutetyl-N',N'-dimethyl-1,3-diaminopropane having a number average molecular weight in the range of from about 600 to about 1500 and (b) an alkylphenyl-poly(oxyalkylene)-N-(2-aminoethyl)carbamate having a number average molecular weight in the range of from about 1400 to about 1800 having at least one basic nitrogen atom and from about 10 to about 25 oxyalkylene groups wherein said alkylphenyl group contains from 1 to about 30 carbons atoms, said oxyalkylene groups contain from about 2 to about 5 carbon atoms and wherein the weight ratio of said N-polyisobutetyl-N',N'-dimethyl-1,3-diaminopropane to said alkylphenyl-poly(oxyalkylene)-N-(2-aminoethyl)carbamate ranges from about 3:1 to about 1:2.

37. An unleaded fuel composition comprising a major amount of a hydrocarbon base fuel of the gasoline boiling range containing an effective amount to reduce intake valve deposits in electronic port fuel injected engines of about 200 ppmw based on the fuel composition of a mixture of (a) a N-polyisobutetyl-N',N'-dimethyl-1,3-diaminopropane having a number average molecular weight in the range of from about 600 to about 1500 and (b) an alkylphenyl-poly(oxyalkylene)-N-(2-aminoethyl)carbamate having a number

average molecular weight in the range of from about 1400 to about 1800 having at least one basic nitrogen atom and from about 10 to about 25 oxyalkylene groups wherein said alkylphenyl group contains from 1 to about 30 carbons atoms, said oxyalkylene groups contain from about 2 to about 5 carbon atoms and wherein the weight ratio of said N-polyisobutetyl-N',N'-dimethyl-1,3-diaminopropane to said alkylphenyl-poly(oxyalkylene)-N-(2-aminoethyl)carbamate is about 3:1.

38. An unleaded fuel composition comprising a major amount of a hydrocarbon base fuel of the gasoline boiling range containing an effective amount to reduce intake valve deposits in electronic port fuel injected engines of about 200 ppmw based on the fuel composition of a mixture of (a) a N-polyisobutetyl-N',N'-dimethyl-1,3-diaminopropane having a number average molecular weight in the range of from about 600 to about 1500 and (b) an alkyl phenyl-poly(oxyalkylene)-N-(2-aminoethyl)carbamate having a number average molecular weight in the range of from about 1400 to about 1800 having at least one basic nitrogen atom and from about 10 to about 25 oxyalkylene groups wherein said alkylphenyl group contains from 1 to about 30 carbons atoms, said oxyalkylene groups contain from about 2 to about 5 carbon atoms and wherein the weight ratio of said N-polyisobutetyl-N',N'-dimethyl-1,3-diaminopropane to said alkylphenyl-poly(oxyalkylene)-N-(2-aminoethyl)carbamate is about 1:1.

39. An unleaded fuel composition comprising a major amount of a hydrocarbon base fuel of the gasoline boiling range containing an effective amount to reduce intake valve deposits in electronic port fuel injected engines of about 250 ppmw based on the fuel composition of a mixture of (a) a N-polyisobutetyl-N',N'-dimethyl-1,3-diaminopropane having a number average molecular weight in the range of from about 600 to about 1500 and (b) an alkylphenyl-poly(oxyalkylene)-N-(2-aminoethyl)carbamate having a number average molecular weight in the range of from about 1400 to about 1800 having at least one basic nitrogen atom and from about 10 to about 25 oxyalkylene groups wherein said alkylphenyl group contains from 1 to about 30 carbons atoms, said oxyalkylene groups contain from about 2 to about 5 carbon atoms and wherein the weight ratio of said N-polyisobutetyl-N',N'-dimethyl-1,3-diaminopropane to said alkylphenyl-poly(oxyalkylene)-N-(2-aminoethyl)carbamate is about 1:1.

40. A method for operating an electronic port fuel injected engine on an unleaded fuel composition compatible with carburetor and throttle body injected engines which comprises introducing into an electronic port fuel injected engine with the combustion intake charge about 200 ppmw based on the fuel composition to reduce intake valve deposits of a mixture of (a) a N-polyisobutetyl-N',N'-dimethyl-1,3-diaminopropane having a number average molecular weight in the range of from about 600 to about 1500 and (b) an alkylphenyl-poly(oxyalkylene)-N-(2-aminoethyl)carbamate having a number average molecular weight in the range of from about 1400 to about 1800 having at least one basic nitrogen atom and from about 10 to about 25 oxyalkylene groups wherein said alkylphenyl group contains from 1 to about 30 carbons atoms, said oxyalkylene groups contain from about 2 to about 5 carbon atoms and wherein the weight ratio of said N-polyisobutetyl-N',N'-dimethyl-1,3-diaminopropane to said alkylphenyl-poly(oxyalkylene)-N-(2-aminoethyl)carbamate is about 3:1.

41. A method for operating an electronic port fuel injected engine on an unleaded fuel composition compatible with carburetor and throttle body injected engines which com-

prises introducing into an electronic port fuel injected engine with the combustion intake charge about 200 ppmw based on the fuel composition to reduce intake valve deposits of a mixture of (a) a N-polyisobutetyl-N',N'-dimethyl-1,3-diaminopropane having a number average molecular weight in the range of from about 600 to about 1500 and (b) an alkylphenyl-poly(oxyalkylene)-N-(2-aminoethyl)carbamate having a number average molecular weight in the range of from about 1400 to about 1800 having at least one basic nitrogen atom and from about 10 to about 25 oxyalkylene groups wherein said alkylphenyl group contains from 1 to about 30 carbons atoms, said oxyalkylene groups contain from about 2 to about 5 carbon atoms and wherein the weight ratio of said N-polyisobutetyl-N',N'-dimethyl-1,3-diaminopropane to said alkylphenyl-poly(oxyalkylene)-N-(2-aminoethyl)carbamate is about 1:1.

42. A method for operating an electronic port fuel injected engine on an unleaded fuel composition compatible with carburetor and throttle body injected engines which comprises introducing into an electronic port fuel injected engine with the combustion intake charge about 250 ppmw based on the fuel composition to reduce intake valve deposits of a mixture of (a) a N-polyisobutetyl-N',N'-dimethyl-1,3-diaminopropane having a number average molecular weight in the range of from about 600 to about 1500 and (b) an alkylphenyl-poly(oxyalkylene)-N-(2-aminoethyl)carbamate having a number average molecular weight in the range of from about 1400 to about 1800 having at least one basic nitrogen atom and from about 10 to about 25 oxyalkylene groups wherein said alkylphenyl group contains from 1 to about 30 carbons atoms, said oxyalkylene groups contain from about 2 to about 5 carbon atoms and wherein the weight ratio of said N-polyisobutetyl-N',N'-dimethyl-1,3-diaminopropane to said alkylphenyl-poly(oxyalkylene)-N-(2-aminoethyl)carbamate is about 1:1.

43. An unleaded fuel composition comprising a major amount of a hydrocarbon base fuel of the gasoline boiling range containing an effective amount to reduce intake valve deposits in electronic port fuel injected engines of from about 50 ppmw to about 500 ppmw based on the fuel composition of a mixture of (a) a Mannich polyamine comprising the condensation product of a high molecular weight sulfur-free alkyl-substituted hydroxyaromatic compound wherein the alkyl group has a number average

molecular weight from about 750 to about 1200, an amine which contains an amino group having at least one active hydrogen atom, and an aldehyde, wherein the respective molar ratio of reactants is 1:0.1-10:0.1-10 and (b) an alkylphenyl-poly(oxyalkylene)-N-(2-aminoethyl)carbamate having a number average molecular weight in the range of from about 1400 to about 1800 having at least one basic nitrogen atom and from about 10 to about 25 oxyalkylene groups wherein said hydrocarbyl group contains from 1 to 30 carbon atoms, and said oxyalkylene groups contain from about 2 to about 5 carbon atoms and wherein the weight ratio of said Mannich polyamine to said alkylphenyl-poly(oxyalkylene)-N-(2-aminoethyl)carbamate is about 1:1.

44. The fuel composition of claim 43 wherein the weight of the mixture of polyamine and aminocarbamate is about 250 ppmw.

45. A method for operating an electronic port fuel injected engine on an unleaded fuel composition compatible with carburetor and throttle body injected engines which comprises introducing into an electronic port fuel injected engine with the combustion intake charge an amount from about 50 ppmw to about 500 ppmw to reduce intake valve deposits of a mixture of (a) a Mannich polyamine comprising the condensation product of a high molecular weight sulfur-free alkyl-substituted hydroxyaromatic compound wherein the alkyl group has a number average molecular weight from about 750 to about 1200, an amine which contains an amino group having at least one active hydrogen atom, and an aldehyde, wherein the respective molar ratio of reactants is 1: 0.1-10:0.1-10 and (b) an alkylphenyl-poly(oxyalkylene)-N-(2-aminoethyl)carbamate having a number average molecular weight in the range of from about 1400 to about 1800 having at least one basic nitrogen atom and from about 10 to about 25 oxyalkylene groups wherein said hydrocarbyl group contains from 1 to 30 carbon atoms, and said oxyalkylene groups contain from about 2 to about 5 carbon atoms and wherein the weight ratio of said Mannich polyamine to said alkylphenyl-poly(oxyalkylene)-N-(2-aminoethyl)carbamate is about 1:1.

46. The method of claim 45 wherein the weight of the mixture of polyamine and aminocarbamate is about 250 ppmw.

\* \* \* \* \*